

Oct. 1, 1968

D. J. STRATFORD

3,404,048

MAGNESIUM ALLOY

Filed May 11, 1966



Inventor:  
David James Stratford  
By Remon Palmer Stewart  
& Estabrook,  
Attorneys

## 1

3,404,048

## MAGNESIUM ALLOY

David James Stratford, Halesowen, Birmingham, England, assignor to Birmetals Limited, Birmingham, England, a British company

Filed May 11, 1966, Ser. No. 549,316

Claims priority, application Great Britain, May 11, 1965,  
19,757/65  
9 Claims. (Cl. 148—161)

## ABSTRACT OF THE DISCLOSURE

Magnesium alloys containing, in addition to magnesium, 2.0 to 30% zinc and 0.2 to 10% manganese are age-hardened following heat treatment or hot working and rapid cooling by ageing in a first stage at temperature of 60° C. to 90° C. for 3 to 31 hours and in a second stage at a temperature of 120° C. to 270° C. for 1 to 70 hours. The resulting alloys are greatly improved in their proof stress and tensile strength as compared to such alloys that are aged by prior known methods.

The present invention consists in a process of age-hardening an alloy of magnesium containing, in addition to incidental impurities, 2.0 to 30% zinc and 0.2 to 10% manganese after solution heat treatment or hot working and rapid cooling, comprising ageing the alloy in two stages, in a first stage of which the alloy is aged within a lower temperature range and in a second stage of which the alloy is aged within a higher temperature range.

## 2

time in that the time to reach optimum properties increases as ageing temperatures decrease.

Our investigations have shown that the effectiveness of the present ageing process is dependent upon the presence of zinc and manganese in the alloy and their relative proportions. It has been found theoretically that in order to achieve optimum mechanical properties it is required to form the hardening precipitate  $Zn_4Mg_3Mn$  which results from the zinc and manganese present in the alloy. The ratio of zinc to manganese in  $Zn_4Mg_3Mn$  is 4.75 to 1. A balanced alloy would therefore contain zinc and manganese in this ratio. Preferably the zinc content by weight is 4.0 to 10% and the manganese content by weight is 0.8 to 2.0%. The mechanical properties which can be achieved in the manganese base alloys to which the process in accordance with the present invention is applied will be readily appreciated from the results of tests given by way of example below.

Table I below shows the results obtained from samples O, P, Q, R, S and T which contained 6.25% zinc, 1.15% manganese with the balance, excluding impurities, magnesium. Each sample was extruded from a 12 inch diameter cast billet into a 2 inch diameter bar at 380° C., cooled to room temperature in air, solution heat treated for 1½ hours at 420° C. and then water quenched. Sample O was tested immediately after the water quench, sample P was tested after ageing only at 180° C. after quenching and samples Q to T were aged, immediately after quenching, for varying periods at 90° C. and then aged at 180° C. for 16 hours.

TABLE I

| Sample | Condition                                                       | .1% PS,<br>tons/in. <sup>2</sup> | .2% PS,<br>tons/in. <sup>2</sup> | T.S.,<br>tons/in. <sup>2</sup> | Percent<br>elongation |
|--------|-----------------------------------------------------------------|----------------------------------|----------------------------------|--------------------------------|-----------------------|
| O      | Solution heat treated and water quenched                        | 12.0                             | 12.7                             | 18.7                           | 17                    |
| P      | As Sample O plus 16 hours at 180° C.                            | 20.4                             | 21.1                             | 23.7                           | 10                    |
| Q      | As Sample O plus 4 hours at 90° C. plus 16 hours<br>at 180° C.  | 21.5                             | —                                | 25.0                           | 8                     |
| R      | As Sample O plus 8 hours at 90° C. plus 16 hours<br>at 180° C.  | 22.1                             | 22.8                             | 25.1                           | 9                     |
| S      | As Sample O plus 24 hours at 90° C. plus 16 hours<br>at 180° C. | 21.9                             | 23.0                             | 25.0                           | 9                     |
| T      | As Sample O plus 31 hours at 90° C. plus 16 hours<br>at 180° C. | 22.1                             | 23.1                             | 25.2                           | 6                     |

By the ageing process according to the present invention it is possible to achieve better mechanical properties in an alloy of the kind described than are possible by normal, single stage, ageing processes. It is also possible to obtain equivalent and better values than those which can be obtained by conventional ageing in appreciably less time.

The ageing process is applicable to the magnesium base alloys in cast or wrought form. As in the case of a single stage ageing process it is essential that hot working or solution heat treatment of the alloy should be followed immediately afterwards by rapid cooling because the mechanical properties which can be achieved by the present ageing process are influenced by the rate of cooling after hot working or solution heat treatment in that improved properties result from high cooling rates. The desired rapid cooling may be achieved by quenching in water or even cooling in air, depending upon the cross-sectional dimensions of the alloy article.

Tests have shown that the greater the difference between the ageing temperatures of the two stages when the ageing temperature of one of the stages is unchanged, preferably the ageing temperature of the second stage, the better are the mechanical properties which can be achieved.

It has been observed that the mechanical properties improve as the temperature of ageing in each of the two stages is lowered. As in a normal, single stage, ageing process there is a relationship between temperature and

45 The percentage elongation given in the results and those below are on  $4\sqrt{A}$  where A is the initial cross-sectional area of the rest piece.

50 The results in the table show that the proof stress and tensile strength of the samples treated in accordance with the present invention are notably higher than for those which can be reached by ageing in the usual way. It will be observed that the tensile strength achieved notably high values after ageing in the first stage for only 4 hours at 90° C.

55 When the ageing temperature of the second stage is 180° C. the alloy is preferably maintained at that temperature for approximately 16 hours, as has been the case in the examples given above. However when an alloy is aged in the first stage at 90° C. and then at 180° C. in the second stage it is possible to achieve noteworthy mechanical properties after ageing for as little as 4 hours at 180° C. as will be shown later.

60 With the magnesium base alloys to which the two stage ageing process herein disclosed is applied, it is possible to obtain high mechanical properties by subjecting the alloys to a normal, single stage, ageing but lengthy periods of time are required. Such mechanical properties and better can be attained in considerably less time by ageing in two stages. This is illustrated by the graph shown in FIGURE 1 of the accompanying drawings which shows the effect of the second stage ageing temperature on the maximum mechanical properties which can be attained in a magnesium alloy with two stage ageing and, for com-

parison, the effect of ageing at those temperatures in a single stage ageing process. The curves on the graph were plotted from results obtained from samples which contained 6.2% zinc, 1.13% manganese with the balance, apart from impurities, magnesium. Each sample was in the form of a 2 inch diameter bar which before ageing was

6.23% zinc and 1.41% manganese with the balance, excluding impurities, magnesium. Each sample before ageing was extruded from a 12 inch diameter billet to a 2 inch diameter bar at 380° C. in a container at 380° C. in a container at 380° C. at 2 feet/minute, solution heat treated for 2 hours at 420° C. and then water quenched.

TABLE III

| Sample | Condition                                            | .1% PS,<br>tons/in. <sup>2</sup> | .2% PS,<br>tons/in. <sup>2</sup> | T.S.,<br>tons/in. <sup>2</sup> | Percent<br>elongation |
|--------|------------------------------------------------------|----------------------------------|----------------------------------|--------------------------------|-----------------------|
| U      | Aged for 24 hours at 90° C. plus 16 hours at 180° C. | 22.1                             | 22.8                             | 25.0                           | 7                     |
| V      | Aged for 24 hours at 60° C. plus 16 hours at 180° C. | 22.5                             | 23.2                             | 25.4                           | 7                     |
| W      | Aged for 24 hours at 90° C. plus 32 hours at 120° C. | 22.9                             | 23.7                             | 25.0                           | 6                     |
| X      | Aged for 24 hours at 60° C. plus 32 hours at 120° C. | 23.9                             | 24.4                             | 26.0                           | 5                     |
| Y      | Aged for 24 hours at 90° C. plus 16 hours at 150° C. | 23.8                             | 24.6                             | 25.8                           | 6                     |
| Z      | Aged for 24 hours at 60° C. plus 16 hours at 150° C. | 24.0                             | 24.8                             | 26.1                           | 7                     |

solution treated for 2 hours at 420° C. and then water quenched. In the graph the curve of .1% proof stress for the single aged samples is represented by a broken line, the curve of tensile strength is represented by a dotted line and the curves of .1% proof stress and tensile strength for the samples aged in two stages are represented respectively by a full line and a chain-dotted line. The times in hours to reach maximum values at particular temperatures are indicated on the .1% proof stress curves. On the two stage ageing curves the times given are the total of the times in the two ageing stages as given in the following Table II:

TABLE II

Total time of ageing = ageing in first stage + ageing in second stage:

86 hours = 16 hours at 60° C. + 70 hours at 120° C.  
20 hours = 4 hours at 90° C. + 16 hours at 150° C.  
8 hours = 4 hours at 90° C. + 4 hours at 180° C.  
6 hours (1) = 4 hours at 90° C. + 2 hours at 210° C.  
6 hours (2) = 4 hours at 90° C. + 2 hours at 240° C.  
4 hours = 3 hours at 90° C. + 1 hour at 270° C.

The effect of ageing temperature on the percent elongation of the alloy with single and two stage ageing is shown by curves Y and Z respectively of the graph.

It will be seen from the graph of FIGURE 1 that whereas, in the temperature range in which the alloy sample was aged, it was necessary with single ageing to age for 142 hours to reach the maximum possible values for .1% proof stress and tensile strength, similar values were reached with the two stage ageing process in less than 20 hours and even higher values were obtained by two stage ageing in a shorter time than was necessary to obtain the maximum properties by single ageing. The above Table II and

There is an improvement in the mechanical properties as the proportion of zinc and manganese which is in the ratio 4.75 to 1, as theoretically required to form the hardening precipitate  $Zn_4Mg_3Mn$ , increases. The linear form 20 of the ageing response curve in relation to alloys containing increasing amounts of zinc and manganese in this ratio is shown clearly by the graph of FIGURE 2 of the accompanying drawings. The curves of the graph of FIGURE 2 were drawn from the results obtained from samples which after solution heat treatment at 420° C. were aged for 24 hours at 90° C. and then for 16 hours at 180° C. The curve of tensile strength in the graph is represented by a full line, the .1% proof stress curve is represented by a chain-dotted line and the .2% proof stress curve is represented by a broken line.

The effect of the ageing process according to the present invention has so far been exemplified only in relation to the magnesium base alloys in wrought form. It is possible, however, to obtain high mechanical properties in cast alloys by two-stage ageing. This is shown in Table IV by the results which were obtained from cast samples Ac and Bc containing by weight 5.46% zinc and 1.1% manganese with the balance, excluding impurities, magnesium. The samples were grain refined using hexachloroethane, sand cast into British D.T.D. Aircraft Standard test bars from which 0.64 inch diameter tensile test pieces were machined, solution treated for 12 hours at 340° C. plus 4 hours at 370° C. and plus 8 hours at 420° C., and then in the case of sample Ac air cooled and in the case of sample Bc quenched in boiling water. Each sample was tested immediately after cooling from the solution heat treatment and again after it was subjected to an ageing process consisting of 30 hours at 60° C. followed by 50 hours at 120° C.

TABLE IV

| Sample | Condition                                                                                        | .1% PS,<br>tons/in. <sup>2</sup> | .2% PS,<br>tons/in. <sup>2</sup> | T.S.,<br>tons/in. <sup>2</sup> | Percent<br>elongation |
|--------|--------------------------------------------------------------------------------------------------|----------------------------------|----------------------------------|--------------------------------|-----------------------|
| Ac     | Air cooled after solution treatment                                                              | 4.3-4.6                          | 5-5.2                            | 11.5-12.5                      | 6-8                   |
| Ac     | Air cooled after solution treatment plus 30 hours at 60° C. plus 50 hours at 120° C.             | 8-8.6                            | 8.9-9.1                          | 11.3-11.8                      | 2-3                   |
| Bc     | Boiling water quenched after solution treatment                                                  | 4-4.5                            | 4.8-5                            | 11-12                          | 6-8                   |
| Bc     | Boiling water quenched after solution treatment plus 30 hours at 60° C. plus 50 hours at 120° C. | 10-10.5                          | 11-11.5                          | 13.5-14                        | 2-3                   |

the graph of FIGURE 1 further show that the lower the temperature of ageing in each of the two stages the higher are the mechanical properties which can be achieved although the time to reach the optimum is increased.

The mechanical properties are also influenced by the difference between the ageing temperatures of the two stages in that the greater the difference between the two ageing temperatures, when one of the temperatures is unchanged, the better are the mechanical properties which can be obtained. This improvement in properties is most apparent when the temperature of the higher temperature ageing stage is maintained constant and the temperature of ageing in the lower temperature stage is varied to increase the temperature difference between the two stages. The effect of the temperature difference will be seen from Table III below in which the results are given of tests made on samples, U, V, W, X, Y and Z which contained

I claim:

60 1. A process of age-hardening a magnesium base alloy after solution heat treatment, or hot working, and rapid cooling, which comprises ageing an alloy which consists of by weight 2.0% to 30% zinc and 0.2% to 10% manganese with the balance, apart from impurities, magnesium, in a first stage in which the alloy is aged for 3 to 31 hours at a substantially constant temperature in the range 60° C. to 90° C. and ageing said alloy in a second stage in which, following directly after the first stage, the alloy is aged for 1 to 70 hours at a substantially constant temperature in the range 120° C. to 270° C.

65 2. A process of age-hardening a magnesium base alloy after solution heat treatment, or hot working, and rapid cooling, which comprises ageing an alloy which consists of by weight 4.0% to 10% zinc and 0.8% to 2.0% manganese with the balance, apart from impurities, magne-

sium, in a first stage in which the alloy is aged for 3 to 31 hours at a substantially constant temperature in the range 60° C. to 90° C. and ageing said alloy in a second stage in which, following directly after the first stage, the alloy is aged for 1 to 70 hours at a substantially constant temperature in the range 120° C. to 270° C.

3. A process according to claim 2 wherein the alloy is aged in the first stage for 24 hours at 90° C. and in the second stage for 32 hours at 120° C.

4. A process according to claim 2 wherein the alloy is aged in the first stage for at least 4 hours at 90° C. and in the second stage for at least 16 hours at 180° C.

5. A process according to claim 2 wherein the alloy is aged in the first stage for at least 3 hours at 90° C. and in the second stage for 1 hour at 270° C.

6. A process according to claim 2 wherein the alloy is aged in the first stage for at least 16 hours at 60° C. and in the second stage for from 32 to 70 hours at 120° C.

7. A process according to claim 2 wherein the alloy is aged in the first stage for at least 24 hours at 60° C. and in the second stage for at least 16 hours at 180° C.

8. A process as claimed in claim 2 wherein said alloy contains by weight 4.0% to 10.0% zinc and 0.8 to 2.0% manganese with the balance, apart from impurities, magnesium and in which alloy the ratio of zinc to manganese is 4.75 to 1.

9. A magnesium base alloy which contains by weight 4.0% to 10% zinc and 0.8% to 2.0% manganese with the balance apart from impurities, magnesium, and the ratio of zinc to manganese in the alloy being 4.75 to 1, prepared by a process as defined in claim 8.

#### References Cited

#### UNITED STATES PATENTS

|    |           |         |             |       |          |
|----|-----------|---------|-------------|-------|----------|
| 15 | 1,886,251 | 11/1932 | Gann        | ----- | 75—168   |
|    | 1,936,550 | 11/1933 | Gann et al. | ----- | 148—161  |
|    | 2,275,188 | 3/1942  | Harrington  | ----- | 148—12.7 |
|    | 2,477,503 | 7/1949  | Vargo       | ----- | 148—161  |

20 CHARLES N. LOVELL, Primary Examiner.